

April 14, 1942.

J. A. LEERMAKERS ET AL

2,279,406

COLOR PROCESS USING CELLULOSE ESTER EMULSIONS

Filed Dec. 26, 1940



JOHN A. LEERMAKERS  
SCHEURING S. FIERKE

INVENTORS

*Naoton M. Berries,*

BY *R. Frank Smith*  
ATTORNEYS

## UNITED STATES PATENT OFFICE

2,279,406

COLOR PROCESS USING CELLULOSE ESTER  
EMULSIONS

John A. Leermakers and Scheuring S. Fierke,  
Rochester, N. Y., assignors to Eastman Kodak  
Company, Rochester, N. Y., a corporation of  
New Jersey

Application December 26, 1940, Serial No. 371,650  
In Great Britain December 29, 1939

5 Claims. (Cl. 95—7)

This invention relates to color photography and particularly to light sensitive cellulosic emulsions having color formers incorporated therein.

In Mannes and Godowsky U. S. application Serial No. 314,689, filed January 19, 1904, there are described photographic emulsions in which couplers or color-forming compounds are mixed with cellulose esters and the mixture dispersed in gelatino-silver halide emulsions. This method of preparing emulsions for use in color photography depends on the use of immiscible phases so that a dispersion of the cellulose ester in the gelatin can be formed. It cannot be used for the preparation of photographic emulsions in which a cellulose ester is the carrier for the silver halide, since the cellulose ester used to dissolve the gelatin would be soluble in the cellulose ester used to disperse the silver halide and a dispersion of one cellulose ester in the other could not be formed.

It is, therefore, an object of the present invention to provide a method for incorporating couplers or color-forming compounds in cellulose ester emulsions. Other objects will appear from the following description of our invention.

These objects are accomplished by forming a dispersion of the coupler in gelatin and dispersing this dispersion in a water-permeable cellulose organic acid ester containing sensitive silver halide grains.

The single figure of the accompanying drawing is a sectional view of a single layer photographic element formed according to our invention.

The invention relates to colored photographic elements of the type in which a support, which may be of transparent material such as cellulose nitrate or cellulose acetate, or of opaque or translucent material such as paper, carries one or more sensitive photographic emulsions containing silver halide grains dispersed in a cellulose ester. The cellulose ester is one which is permeable to photographic processing baths, such as photographic developing and fixing solutions. In this emulsion there is dispersed gelatin particles containing color-forming or coupling compounds. By reason of the fact that gelatin is water-soluble, it does not mix with the cellulose ester of the silver halide emulsion but, under the proper conditions, forms a dispersion in the sensitive emulsion. The color-forming compounds incorporated in the gelatin particles are of the well-known type containing

reactive methylene or phenolic hydroxyl groups and are capable of combining with the oxidation product of a primary aromatic amino developing agent upon photographic development to form a colored image. Metallic silver is formed simultaneously with the production of the colored image and this silver may be subsequently removed without removal of the dye, leaving substantially clear, transparent dye images.

The cellulose esters suitable for formation of the emulsions used in our invention are preferably hydrolyzed cellulose organic acid esters such as those described in Salo U. S. Patent 2,110,491, granted March 8, 1938. These esters have an acyl content of from about 19% to about 33, preferably 19% to 26%.

Our invention may be used for the formation of photographic images of a single color in a single photographic layer or for the formation of natural color images in multi-layer photographic coatings. The cellulose ester emulsions may be sensitized with optical sensitizers in the well-known manner so that the natural sensitivity of the esters to blue light may be extended into the green and red spectral regions.

Our invention will be understood by reference to the following examples which illustrate the formation of color-forming emulsions according to our invention:

## Example 1

To 200 cc. of a 10% gelatin solution in water there was added 0.8 cc. of sodium hydroxide and to this alkaline gelatin solution there were added with rapid stirring 4 grams of a solution of 2-lauryl-4-chlorophenol in 20 cc. of ethyl alcohol containing 2 cc. of sodium hydroxide. Following the addition of the coupler, 8.4 cc. of citric acid (20% solution) were added. Upon the addition of the acid, the coupler precipitated as fine micro crystals in the gelatin solution. 20 cc. of this dispersion of coupler in gelatin were then added to a photographic silver halide emulsion in which the vehicle was cellulose acetate propionate of 33% acyl content. This emulsion before the addition of the coupler-gelatin dispersion, had the following composition:

|                              |      |       |
|------------------------------|------|-------|
| Ethylene chloride            | cc   | 18    |
| Ethyl alcohol                | cc   | 2     |
| Cellulose acetate propionate | gram | 0.5   |
| Silver bromide               | do   | 0.876 |

After the addition of the gelatin-coupler dispersion, the emulsion was further diluted with 20

cc. of ethylene chloride in order to decrease its viscosity.

Since the coupler incorporated in this emulsion was one capable of producing a blue-green dye upon development in primary aromatic amino developing solutions, the emulsion was rendered sensitive to red light prior to the addition of the coupler-gelatin dispersion. This may be accomplished by the use of any of the well known red sensitizers but in the present case a suitable amount of 5-4-(3-ethyl-2-(3)-benzothiazolilidene)-2-butenyldene-3-n-heptyl-1-phenyl-2-thiohydantoin was used.

After addition of the coupler-gelatin dispersion to the emulsion, the emulsion was passed through a colloid mill or homogenizer to form a dispersion of gelatin in the emulsion and was then coated on a suitable support.

*Example 2*

A green-sensitive emulsion was prepared in the same manner as described in Example 1, except that a green sensitizer and a coupler capable of yielding a magenta dye upon development were used. The emulsion was sensitized to green light with 5-(3-ethyl-2-(3)-benzoxazolylidene)-ethyldene-3-n-heptyl-1-phenyl-2-thiohydantoin. The coupler used in this case was 2-cyanoacetyl-5-(p-sec. amylbenzoyl-amino)-coumarone.

*Example 3*

An emulsion was prepared in the same manner as described in Example 1 except that it was not specially sensitized and a coupler capable of yielding a yellow image upon photographic development was used. In this case the coupler was n-propyl-p-benzoylacetaminobenzene sulfonate.

*Example 4*

In addition to the single layer coatings, the red sensitive emulsion prepared as described in Example 1 was coated on a transparent support and over it there was coated the green sensitive emulsion prepared as described in Example 2. Upon suitable exposure and development this multi-layer coating yielded a blue-green image in the bottom emulsion layer and a magenta image in the top emulsion layer.

Instead of the 33% acyl cellulose acetate propionate described in the examples, the coupler dispersion in gelatin may also be added to a far-hydrolyzed cellulose acetate propionate emulsion in which the acyl content is as low as 19 to 20%. This may be coated either sensitized or un sensitized. The coating thus prepared is much more permeable to water than is that in which the vehicle for the silver halide emulsion is a cellulose organic acid ester of 33% acyl content. However, in the case of the cellulose organic acid esters of 19-20% acyl content, the cellulose ester is more readily precipitated from solution by the addition of water or aqueous solutions so that with this ester the amount of coupler which may be added to the emulsion is of the order of 10 to 20% of that which may be used with the higher acyl cellulose esters.

In the case of the emulsions of higher acyl content whose water permeability is relatively low, porosity modifiers may be added to increase the permeability of the ester to processing solutions and thereby to increase the amount of dye formed. Compounds suitable for this purpose are the porosity modifiers described in Mannes

and Godowsky U. S. application Serial No. 314,689, filed January 19, 1940.

Emulsions made according to our invention may be developed with any suitable solution of a primary aromatic amino developing agent such as p-phenylenediamine and its substituted derivatives. The compounds which we prefer to use are dialkyl-p-phenylene diamines substituted in one amino group, the other amino group remaining unsubstituted. These compounds are ordinarily used in the salt form such as the hydrochloride or sulfate since these compounds are more stable than the amines themselves. Developing agents which may be used include diethyl-p-phenylenediamine, monomethyl-p-phenylenediaminehydrochloride and diethyl-p-phenylenediamine-sulfate.

The developer used for coatings made with low acyl (19-20% content) cellulose acetate propionate-silver halide emulsions may have the following composition:

|                              |         |        |
|------------------------------|---------|--------|
| 2 - amino - 5 - diethylamino | toluene |        |
| HCl                          | grams   | 2.0    |
| Sodium sulfite               | do      | 2.0    |
| Potassium bromide            | do      | 2.0    |
| Sodium carbonate             | do      | 20.0   |
| Water to make                | cc.     | 1000.0 |

This developer was found to produce good color in 10 to 15 minutes' development.

Photographic coatings described in the specific examples using a cellulose acetate propionate of about 33% acyl content require a more energetic developer such as one having the following composition:

|                                  |         |        |
|----------------------------------|---------|--------|
| Sodium sulfite                   | grams   | 15.0   |
| 2 - a m i n o - 5 - diethylamino | toluene |        |
| HCl                              | grams   | 2.0    |
| Kodak                            | do      | 50.0   |
| Sodium hydroxide                 | do      | 0.5    |
| 6-nitrobenzimidazole             | do      | 0.01   |
| Potassium bromide                | do      | 2.0    |
| Water to make                    | cc.     | 1000.0 |

The development time with this developer varied from 10-25 minutes, a shorter time being used for the single layer coatings.

Since the color development fixation and removal of silver from ferricyanide solutions is rather slow in the case of the high acyl cellulose acetate propionate emulsions due to low water permeability the speed of these various processes can be increased by the addition to the developer, a fixing bath or other baths of organic compounds such as benzyl alcohol, acetone, etc. to increase the permeability of these layers.

Reference will now be had to the accompanying drawing which further illustrates our invention. As shown therein, a support 10 of any suitable material such as glass, cellulose ester, synthetic resins or paper, has coated thereon a layer 11 of hydrolyzed cellulose organic acid ester containing silver halide particles 12 and dispersed particles 13 of gelatin containing coupler. Multi-layer coatings may be made in a similar way and may be superimposed on the same side or on opposite sides of a support. In the case of a 3-layer coating of superposed layers on one side of a support the outer layer will usually be blue-sensitive, the middle layer green-sensitive and the innermost layer red sensitive in the well known manner. In this case the customary yellow filter layer will be coated between the blue-sensitive layer and the green-sensitive layer in order to prevent the ac-

tion of blue light on the green sensitive layers and the red sensitive layers during the exposure of the element.

Our process possesses the advantages that diffusion of the couplers in the emulsion may be reduced by incorporating the coupler in gelatin, and fading of the resulting dye images is found to be decreased.

The examples and modifications included in the present specification are illustrative only and modifications may be made in our process without in the scope of the appended claims.

We claim:

1. The method of producing a color-forming photographic layer, which comprises mixing, in alkaline solution, gelatin with a color-forming compound capable of reacting with a primary aromatic amino developing agent on photographic development, acidifying the solution to form a fine dispersion of the color-forming compound in the gelatin, and dispersing the gelatin and color-forming compound in a water-permeable cellulose acetate propionate-silver halide emulsion.

2. The method of producing a color-forming photographic layer, which comprises mixing, in alkaline solution, gelatin with a color-forming compound capable of reacting with a primary aromatic amino developing agent on photographic development, acidifying the solution to form a fine dispersion of the color-forming compound in the gelatin, and dispersing the gelatin and color-forming compound in a water-permeable cellulose organic acid ester-silver halide emulsion.

3. The method of producing a color-forming

photographic layer, which comprises mixing, in alkaline solution, gelatin with a color-forming compound capable of reacting with a primary aromatic amino developing agent on photographic development, acidifying the solution to form a fine dispersion of the color-forming compound in the gelatin, and dispersing the gelatin and color-forming compound in a water-permeable cellulose acetate propionate-silver halide emulsion.

4. The method of producing a color-forming photographic layer, which comprises mixing, in alkaline solution, gelatin with a color-forming compound capable of reacting with a primary aromatic amino developing agent on photographic development, acidifying the solution to form a fine dispersion of the color-forming compound in the gelatin, and dispersing the gelatin and color-forming compound in a water-permeable cellulose acetate propionate of approximately 33% acyl content.

5. The method of producing a color-forming photographic layer, which comprises mixing, in alkaline solution, gelatin with a color-forming compound capable of reacting with a primary aromatic amino developing agent on photographic development, acidifying the solution to form a fine dispersion of the color-forming compound in the gelatin, and dispersing the gelatin and color-forming compound in a water-permeable cellulose acetate propionate of approximately 20% acyl content silver halide emulsion.

JOHN A. LEERMAKERS.  
SCHEURING S. FIERKE.